

(No Model.)

J. WALKER.

DEPHOSPHORIZING AND OTHERWISE PURIFYING MOLTEN IRON OR STEEL.

No. 244,696.

Patented July 19, 1881.



Fig. 1.



Fig. 2.

Witnessed  
R. H. Higley  
J. L. Walker

Inventor John Walker  
By Attorney George H. Christy

# UNITED STATES PATENT OFFICE.

JOHN WALKER, OF CLEVELAND, OHIO, ASSIGNOR TO HIMSELF AND  
WILSON B. CHISHOLM, OF SAME PLACE.

## DEPHOSPHORIZING AND OTHERWISE PURIFYING MOLTEN IRON OR STEEL.

SPECIFICATION forming part of Letters Patent No. 244,696, dated July 19, 1881.

Application filed March 24, 1881. (No model.)

To all whom it may concern:

Be it known that I, JOHN WALKER, of Cleveland, county of Cuyahoga, State of Ohio, have invented or discovered a new and useful Improvement in Dephosphorizing and otherwise Purifying Molten Iron or Steel; and I do hereby declare the following to be a full, clear, concise, and exact description thereof, reference being had to the accompanying drawings, making a part of this specification, in which—like letters indicating like parts—

Figure 1 is a vertical sectional view of a box charged with suitable material for dephosphorizing purposes, and illustrative of my present invention, and Fig. 2 is a horizontal sectional view thereof in the plane of the line  $xx$ , Fig. 1.

The fact that various materials, such as alumina, magnesia, &c., are useful elements in the elimination of phosphorus and other impurities in the making of iron, is well known in the art, and in connection with the Bessemer and Siemens-Martin or open-hearth processes, such ingredients have been utilized for such purposes by working them into the linings of the converter or hearth, as in the "basic-lining process," so called. In the use of such or other like purifying agents it is sometimes important that they be so applied that the entire body or mass of the molten metal shall be subject to their action. It is well known that the metal, both in the Bessemer and open-hearth processes, is necessarily at a high temperature, so that even if an amount of dephosphorizing material chemically sufficient be introduced at a single charge it is liable to be fused or gasified, or to go into other combinations, and its dephosphorizing action exhausted before the entire body or mass of the molten metal has been subjected to its action.

By my present invention I inclose the dephosphorizing or other purifying agents in a box or case composed of a series of two or more chambers, preferably one inside the other, in such manner that the inclosing-walls of the several chambers shall be successively fused at different times, one after another, and thereby different portions of the entire charge shall successively be brought into contact or intermixture with the molten metal, whereby the process of dephosphorization and elimination of

other impurities shall be carried on more slowly and under such conditions that all, or substantially all, parts of the molten metal shall be subjected to the action of the ingredients so introduced.

The box or case A may be made of any suitable material, but for most purposes I prefer cast-iron, both on account of cheapness and because such material may be added to the charge without injury, and sometimes with positive benefit to the product. It may be made of any desired size and proportions; and while I have found that a diameter and height of one foot, with other parts, as shown, proportioned to about the same scale, gives good results, I do not limit myself thereto.

As shown, the box or case consists of a bottom,  $a$ , a cylindrical outer side,  $a'$ , and two concentric inner rings,  $a^2$   $a^3$ , spaced and shaped so as to give a series of chambers,  $b$   $b'$   $b^2$ , into which the dephosphorizing or other purifying ingredients are placed. A lid or cover,  $a^4$ , is then cast on top of the case in such manner—say by bevels, as shown, or otherwise—as to be retained or kept firmly in place. This cover may, however, be made of other material, if so preferred.

Assuming the dephosphorizing process to be employed, and the several chambers  $b$   $b'$   $b^2$  to contain sufficient dephosphorizing material for treating one entire charge of molten metal, the box or case is then at the proper time placed directly into the molten mass. The intense heat will fuse first the outer shell, and then the contents of the outer chamber will unite or intermix with the charge, and by the usual chemical action dephosphorize it in part. At or about the time, as near as may be, that this part of the charge has exhausted its dephosphorizing capacity the next inner shell will be fused, and the contents of chamber  $b'$  will come in contact or be intermixed with the molten mass, so that the dephosphorizing operation will still go on.

In the Bessemer process the violent agitation caused by blowing will so intermix the metal and the dephosphorizing ingredients thus successively brought into action that practically the entire charge will have been subjected to the chemical action indicated by the

time the contents of the innermost chamber,  $b^2$ , shall have exhausted their action; and in the open-hearth process, if the agitation of the metal is not sufficient for this purpose, mechanical means, such as are well known in the art, may be resorted to in order to attain the desired result. Any material suitable for the purpose may be used in the chambers  $b$   $b'$   $b^2$ , such as magnesian limestone having a considerable percentage of magnesia—say thirty to forty per centum, more or less—with or without the alumina.

If limestone having the requisite percentage of magnesia is not obtainable, an artificial compound may be used; but as regards material, I do not limit myself to any particular mixture or natural product, provided only it be suitable for the purpose.

If the charge be so large, or the capacity of the case employed be so small that the contents of one case will be insufficient to complete the work desired, two or more cases may be employed, one being put in first and one or more afterward, in succession, at about such intervals as will allow for the full action of the contents of the previous case; but I believe the better plan to be to have a sufficient number of chambers, and of sufficient capacity in each case, so that the desired chemical action in any one charge of molten metal shall be practically accomplished thereby; also, the relative thicknesses of the successive shells, as well as the relative capacities of the successive chambers formed thereby, may be varied at pleasure, with reference to securing the fusion of the shells and the chemical actions indicated at such stages of the conversion of the metal, as may be preferred, since it is generally believed that the facility or ease with which phosphorus can be eliminated varies somewhat with the varying temperature and condition of the metal.

If the skilled worker desires to dephosphorize the metal slowly at first and more rapidly afterward, he will have his cases made with shells which will fuse more rapidly from the outside toward the inside, or with chambers of greater

capacity from the outside toward the inside, and vice versa, or the effect may be varied by varying the ingredients in the different chambers; or all these variable elements of construction and use may be employed at the same time with reference to getting the best results, as the skilled worker may prefer; also, the cases, instead of being cylindrical, may be made rectangular or of other desired shape, with dividing walls or partitions varying in thickness or relative arrangement, such that the materials contained in the series or "nest" of chambers so formed will, by the successive fusing of the outer and dividing walls or partitions, be brought in succession, one after another, into contact or intermixture with the molten metal; and while I have shown a three-chamber case, the number of chambers may be varied at pleasure, from two upwardly. For most purposes I believe that three or four will be the best number; and for the elimination of other impurities than phosphorus, the like means may be employed, with the mere change of the material inclosed in the chambers of the case, which should always be such as adapted to do the work desired under the conditions named.

I claim herein as my invention—

1. The method of introducing dephosphorizing or other purifying ingredients in successive measured quantities into a charge of molten metal by inclosing such measured quantities in a series or nest of chambers, the inclosing walls of which are successively fusible, and introducing such nest directly into the molten charge, substantially as set forth.

2. A close metallic case, A, having one or more inner rings,  $a^2$   $a^3$ , and filled in the chambers  $b$   $b^2$  with dephosphorizing or other purifying ingredients, substantially as described.

In testimony whereof I have hereunto set my hand.

JOHN WALKER.

Witnesses:

W. R. PALMER,  
JAMES GIBB.